



US005364754A

**United States Patent** [19]

Kim et al.

[11] **Patent Number:** 5,364,754[45] **Date of Patent:** \* Nov. 15, 1994

[54] **SILVER HALIDE PHOTOGRAPHIC EMULSIONS PRECIPITATED IN THE PRESENCE OF ORGANIC DICHALCOGENIDES**

[75] Inventors: **Sang H. Kim**, Pittsford; **Anthony Adin**; **Richard E. Beal**, both of Rochester; **Jerzy A. Budz**, Fairport; **Wai K. Lam**; **Mark A. Whitson**, both of Webster, all of N.Y.

[73] Assignee: **Eastman Kodak Company**, Rochester, N.Y.

[\*] Notice: The portion of the term of this patent subsequent to Jun. 8, 2010 has been disclaimed.

[21] Appl. No.: 968,548

[22] Filed: Oct. 29, 1992

**Related U.S. Application Data**

[63] Continuation-in-part of Ser. No. 869,670, Apr. 16, 1992, abandoned.

[51] **Int. Cl.<sup>5</sup>** ..... G03C 1/34; G03C 1/015; G03C 1/005

[52] **U.S. Cl.** ..... 430/569; 430/567; 430/607; 430/611; 430/613; 430/614

[58] **Field of Search** ..... 430/611, 607, 608, 546, 430/567, 569, 613, 614

[56] **References Cited**

**U.S. PATENT DOCUMENTS**

1,962,133 6/1934 Brooker et al. ..... 430/611  
2,465,149 3/1949 Dersch et al. .....  
2,756,145 7/1956 Ballard et al. ..... 430/607

2,948,614 8/1960 Allen et al. ..... 430/446  
3,043,696 7/1962 Herz et al. ..... 430/603  
3,057,725 10/1962 Herz et al. ..... 430/611  
3,062,654 11/1962 Allen et al. ..... 430/603  
3,128,186 4/1964 Corben et al. ..... 430/611  
3,397,986 8/1968 Millikan et al. ..... 430/603  
3,563,754 2/1971 Jones et al. ..... 430/570  
4,006,025 2/1977 Swank et al. ..... 430/580  
4,379,837 4/1983 Lapp et al. ..... 430/434  
4,468,454 8/1984 Brown ..... 430/569  
4,474,872 10/1984 Onishi et al. ..... 430/512  
4,607,000 8/1986 Gunther ..... 430/428  
4,713,322 12/1987 Bryan et al. ..... 430/569  
4,749,646 6/1988 Herz et al. ..... 430/569  
4,826,758 5/1989 Yoshida et al. ..... 430/569  
4,912,017 3/1990 Takagi et al. ..... 430/264  
5,217,859 6/1993 Boettcher et al. ..... 430/569  
5,219,721 6/1993 Klaus et al. ..... 430/569  
5,229,264 7/1993 Pätzold et al. ..... 430/567

*Primary Examiner*—Charles L. Bowers, Jr.

*Assistant Examiner*—Mark F. Huff

*Attorney, Agent, or Firm*—Sarah Meeks Roberts

[57]

**ABSTRACT**

This invention provides a method of preparing a silver halide photographic emulsion which comprises adding to the silver halide emulsion before or during precipitation a non-labile chalcogen compound represented by Formula I:

$$R^1-X^1-X^2-R^2 \quad (\text{Formula I})$$

It further provides a silver halide photographic emulsion prepared by the above method.

**18 Claims, No Drawings**

**SILVER HALIDE PHOTOGRAPHIC EMULSIONS  
PRECIPITATED IN THE PRESENCE OF ORGANIC  
DICHALCOGENIDES**

This application is a continuation-in-part of co-pending U.S. application Ser. No. 07/869,670 filed Apr. 16, 1992, now abandoned.

**FIELD OF THE INVENTION**

This present invention relates to light sensitive silver halide emulsions. In particular, it relates to light sensitive silver halide emulsions precipitated in the presence of organic dichalcogenides.

**BACKGROUND OF THE INVENTION**

Problems with fogging have plagued the photographic industry from its inception. Fog is a deposit of silver or dye that is not directly related to the image-forming exposure, i.e., when a developer acts upon an emulsion layer, some reduced silver is formed in areas that have not been exposed to light. Fog can be defined as a developed density that is not associated with the action of the image-forming exposure, and is usually expressed as "D<sub>min</sub>", the density obtained in the unexposed portions of the emulsion. A density, as normally measured, includes both that produced by fog and that produced by exposure to light.

It is known in the art that the appearance of photographic fog related to reduction of silver ion can occur during many stages of preparation of the photographic element including silver halide emulsion preparation, (spectral) chemical sensitization of the silver halide emulsion, melting and holding of the liquid silver halide emulsion melts, subsequent coating of silver halide emulsions, and prolonged natural and artificial aging of coated silver halide emulsions. Particularly, silver halide emulsions precipitated in the presence of ripeners such as thioethers or ammonia and/or in environments sensitive to reduction of silver ions such as high pH and/or low pAg usually suffer from high fog and poor raw stock keeping (RSK).

Several methods have been employed to minimize this appearance of fog. Mercury containing compounds, such as those described in U.S. Pat. Nos. 2,728,663; 45 2,728,664; and 2,728,665, have been used as additives to combat fog. Thiosulfonate and thiosulfonate esters, such as those described in U.S. Pat. Nos. 2,440,206; 2,934,198; 3,047,393; and 4,960,689, have also been employed.

Aromatic, heterocyclic, and acyclic disulfides which do not have labile sulfur or sulfide, such as those described in U.S. Pat. Nos. 1,962,133; 2,465,149; 2,756,145; 3,043,696; 3,057,725; 3,062,654; 3,128,186; and 3,563,754, have been used primarily as emulsion melt additives, i.e., being introduced into already (spectral) chemically sensitized silver halide emulsions prior to coating. U.S. Pat. No. 3,397,986 discloses bis(4-acylamidophenyl)disulfides as useful antifoggants added before or after any optically sensitizing dyes. However, the use of optically sensitizing dyes during chemical sensitization was not readily known in the art until their widespread use during tabular shaped silver halide emulsion sensitization. U.S. Pat. No. 3,397,986 and the others cited previously did not anticipate the utility of these non-labile disulfides during the sensitization of silver halide emulsions, either with or without optically sensitizing dyes. The prior art use of these

disulfides as melt additives does decrease fog and stabilize against fog during aging of coated emulsions, but when used in this manner also decreases sensitivity and requires the use of additional stabilizers like azaindenes, 5 such as described in U.S. Pat. No. 3,859,100.

Another challenge in the manufacture of photographic emulsions is the control of the shape and size of the silver halide grains. Morphology (crystal shape) of silver halide emulsion grains plays an important role in 10 their photographic applications. For example, high aspect ratio tabular grain silver halide emulsions have been recognized to provide a variety of photographic advantages, such as improved speed-granularity relationships, increased image sharpness, 15 and reduced blue speed of minus blue recording emulsion layers as illustrated in Kofron et al, U.S. Pat. No. 4,439,520. Research Disclosure 25330, published by Kenneth Mason Publications, Ltd., Dudley Annex, 12a North Street, Emsworth, Hampshire P010 7DQ, ENGLAND, by Buhr et al, discloses how to utilize optical properties of tabular emulsions for optimizing photographic responses of specific layers depending on their grain thicknesses.

Silver chloride crystals are mostly of cubic morphology bound by (100) faces when precipitated under standard conditions. In some cases, other faces may appear. It is most common, however, that (111) and perhaps (110) crystallographic faces occupy only a small fraction of the total crystal surface. The relative amount of those faces may depend on the presence of selective growth modifiers, which would be able to slow down the growth of fast growing faces like (111) and (110). Such growth modifiers are known in the art; W. Reinders, "Study of Photohalides III, Absorption of Dyes, Proteins, and Other Organic Compounds in Crystalline Silver Chloride", *Zeitschrift fur Physikalische Chemie*, volume 77, pages 677-699 (1911), J. Maskaski CA 1,280,312 and references therein. It is also known that different crystallographic faces respond differently to chemical sensitization. Therefore, it is desirable to be able to control some aspects of chemical sensitization with crystal morphology.

T. H. James, "The Theory of the Photographic Process", pages 98-100, Fourth Edition, Macmillan Publishing Company, Inc., New York (1977), describes how various crystal morphologies are formed in different grain formation conditions such as in an excess of bromide ions and solvents such as ammonia. As an example, AgBrI emulsions can be made in various morphologies depending on pAg (silver ion activity). "Particle growth in Suspensions", page 159, Academic Press, London, (1973), discusses growth modifying agents including cationic surfactants and thioureas as growth accelerators and 1-phenyl-5-mercaptopentrazole (PMT), 4-hydroxy-6-methyl-1,3,3a,7-tetraazaindene (TAI) and certain cyanine dyes as growth restrainers. U.S. Pat. No. 4,749,646 (Herz et al) discloses the use of a 1,1,3,3-tetrasubstituted middle chalcogen urea compound as an effective grain growth modifying agent.

U.S. Pat. No. 4,912,017 (Y. Takagi and S. Nishiyama) discloses the use of sulfur-containing compounds such as PMT and mercaptothiadiazoles and thio-ketone group containing compounds to prevent grain size fluctuation (development unevenness) after formation of grains. It also discloses the use of disulfide compounds which are easily cleavable into the above compounds. These compounds can allegedly adsorb to the surface of silver halide crystals. This patent teaches that the pre-

ferred point of addition is during the preparation of a diluted coating emulsion.

There is a continuing need for methods of improving the fog characteristics of photographic emulsions. Further, there is a continuing need for additional methods of controlling grain formation to improve photoefficiency. In accordance with this invention, it has been found that the addition of certain organic dichalcogenides during precipitation of a silver halide emulsion can modify the grain growth of silver halide crystals. This allows the independent control of surface morphology, thickness, size, and dispersity.

It has also been found that the addition of these same dichalcogenide compounds to a silver halide emulsion during precipitation gives lower fog without a concomitant large loss in sensitivity. It has further been found that equivalent fog reduction can be obtained with less dichalcogenide when the dichalcogenide is used during precipitation, rather than as a melt additive, and that less or no latent image destabilization occurs. Additionally, less loss in sensitivity occurs after aging of the coated emulsions.

#### SUMMARY OF THE INVENTION

This invention provides a method of making a photographic silver halide emulsion comprising precipitating a silver halide emulsion and adding to the silver halide emulsion before or during precipitation a non-labile chalcogen compound represented by Formula I:



where  $X^1$  and  $X^2$  are independently S, Se, or Te; and  $R^1$  and  $R^2$ , together with  $X^1$  and  $X^2$ , form a ring system, or are independently substituted or unsubstituted cyclic, acyclic or heterocyclic groups.

In one embodiment, the dichalcogenide compound is a disulfide compound represented by Formula II or III.



(Formula II)

In Formula II, G is independently in an ortho, meta, or para position on the aromatic nucleus relative to the sulfur and is hydrogen, hydroxy,  $\text{SO}_3\text{M}$  or  $\text{NR}^3\text{R}^4$ ,

$\text{M}$  is hydrogen, or an alkaline earth, alkylammonium or arylammonium cation;

$\text{R}^3$  is hydrogen, or a substituted or unsubstituted alkyl or aryl group;

$\text{R}^4$  is hydrogen,  $\text{O}=\text{C}-\text{R}^5$ , or  $\text{O}=\text{C}-\text{N}-\text{R}^6\text{R}^7$ ; and

$\text{R}^5$ ,  $\text{R}^6$ , and  $\text{R}^7$  are independently hydrogen, or hydroxy, or an unsubstituted alkyl, or aryl group, or a substituted or unsubstituted fluoroalkyl, fluoroaryl, carboxyalkyl, carboxyaryl, alkylthioether, arylthioether, sulfoalkyl, or sulfoaryl group or the free acid, alkaline earth salt or alkylammonium or arylammonium salt of the aforementioned groups.

(Formula III)



5

In Formula III, Z contains substituted or unsubstituted carbon or hetero atoms sufficient to form a ring; and  $\text{R}^8$  is a substituted or unsubstituted alkyl or aryl group of 2 to 10 carbon atoms, or the free acid, alkaline earth salt, arylammonium or alkylammonium salt of the aforementioned groups.

In other embodiments, the silver halide emulsion may be a reduction sensitized or a doped emulsion. In a further embodiment, the dichalcogenide compound is added to the silver halide emulsion as a solid particle dispersion.

This invention further provides a photographic silver halide emulsion prepared by the method described above.

#### DETAILED DESCRIPTION OF THE INVENTION

The dichalcogenic compounds of this invention are represented by Formula I:



In the above formula,  $X^1$  and  $X^2$  are independently S, Se, or Te; and  $R^1$  and  $R^2$ , together with  $X^1$  and  $X^2$ , form a ring system, or are independently substituted or unsubstituted cyclic, acyclic or heterocyclic groups. Preferably, the molecule is symmetrical and  $R^1$  and  $R^2$  are alkyl or aryl groups. Preferred is the combination of  $R^1$  and  $R^2$  resulting in a dichalcogenide with a molecular weight greater than 210 g/mol.  $R^1$  and  $R^2$  cannot be groups which cause the compound to become labile, such as, for example,



30

35

40

45

50

55

Examples of preferred compounds are shown below:

#### EXAMPLES OF FORMULA I



-continued



-continued



20 The dichalcogen must be non-labile, meaning it does not release elemental chalcogen or chalcogen anion under specified conditions for making conventional photographic emulsions or the resulting photographic element.

25 Preferably, the dichalcogenide compound is a disulfide compound represented by Formula II or III.

(Formula II)



30 35 In Formula II, G is independently in an ortho, meta, or para position on the aromatic nucleus relative to the sulfur. More preferably, the molecule is symmetrical and most preferably G is in the para position. G is hydrogen, hydroxy,  $\text{SO}_3\text{M}$  or  $\text{NR}^3\text{R}^4$ . More preferably, G is  $\text{NR}^3\text{R}^4$ .

40 45 50 M is hydrogen, or an alkaline earth, alkylammonium or arylammonium cation. Preferably, M is hydrogen or sodium, and more preferably, M is sodium.  $\text{R}^3$  is hydrogen, or a substituted or unsubstituted alkyl or aryl group. Preferred substituents on the alkyl or aryl groups of  $\text{R}^3$  may be methyl, amino, carboxy, or combinations thereof. The preferred groups contain up to 20, and more preferably, up to 10 carbon atoms. Examples of suitable groups are trifluoromethyl, methyl, ethyl, propyl, phenyl, and tolyl.

55 60 65  $\text{R}^4$  is hydrogen,  $\text{O}=\text{C}-\text{R}^5$ , or  $\text{O}=\text{C}-\text{N}-\text{R}^6\text{R}^7$ . More preferably,  $\text{R}^4$  is hydrogen, or  $\text{O}=\text{C}-\text{R}^5$ .

65 70 75  $\text{R}^5$ ,  $\text{R}^6$ , and  $\text{R}^7$  are independently hydrogen, or hydroxy, or an unsubstituted alkyl, or aryl group, or a substituted or unsubstituted fluoroalkyl, fluoroaryl, carboxyalkyl, carboxyaryl, alkylthioether, arylthioether, sulfoalkyl, or sulfoaryl group or the free acid, alkaline earth salt or alkylammonium or arylammonium salt of the aforementioned groups. Examples of suitable groups are trifluoromethyl, methyl, ethyl, n-butyl, isobutyl, phenyl, naphthyl, carboxymethyl, carboxypropyl, carboxyphenyl, oxalate, terephthalate, methylthiomethyl, and methylthioethyl.

80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 94

bly, the disulfide compound is p-acetamidophenyl disulfide.

Examples of preferred disulfide compounds are listed in Table 1.

TABLE I

| Examples of Formula II* |           |                                                              |
|-------------------------|-----------|--------------------------------------------------------------|
| Designation;            | Position, | Substituent Structure of G                                   |
| II-1                    | para      | N(H)C(O)CH <sub>3</sub>                                      |
| II-2                    | meta      | N(H)C(O)CH <sub>3</sub>                                      |
| II-3                    | ortho     | N(H)C(O)CH <sub>3</sub>                                      |
| II-4                    | para      | NH <sub>2</sub> × HCl                                        |
| II-5                    | para      | N(H)C(O)H                                                    |
| II-6                    | ortho     | N(H)C(O)H                                                    |
| II-7                    | para      | N(H)C(O)CF <sub>3</sub>                                      |
| II-8                    | ortho     | N(H)C(O)CF <sub>3</sub>                                      |
| II-9                    | para      | N(H)C(O)-phenyl                                              |
| II-10                   | para      | N(H)C(O)-ethyl                                               |
| II-11                   | para      | N(H)C(O)-propyl                                              |
| II-12                   | para      | N(H)C(O)-naphthyl                                            |
| II-13                   | para      | N(H)C(O)C <sub>7</sub> H <sub>15</sub>                       |
| II-14                   | para      | N(H)C(O)C <sub>14</sub> H <sub>29</sub>                      |
| II-15                   | para      | N(H)C(O)C <sub>17</sub> H <sub>35</sub>                      |
| II-16                   | para      | N(H)C(O)CH <sub>2</sub> -S-C <sub>12</sub> H <sub>25</sub>   |
| II-17                   | para      | N(H)C(O)CH <sub>2</sub> -S-CH <sub>3</sub>                   |
| II-18                   | para      | N(H)C(O)C <sub>2</sub> H <sub>4</sub> -S-CH <sub>3</sub>     |
| II-19                   | para      | N(H)C(O)CH <sub>2</sub> (CH <sub>3</sub> )-S-CH <sub>3</sub> |
| II-20                   | para      | N(H)C(O)-phenyl(2-SO <sub>3</sub> Na)                        |
| II-21                   | para      | N(H)C(O)C(CH <sub>3</sub> ) <sub>3</sub>                     |
| II-22                   | para      | N(H)C(O)-phenyl(4-CO <sub>2</sub> CH <sub>3</sub> )          |

\*atoms in parentheses in structure indicate they are substituted to the atom on the left.



(Formula III)

In Formula III, Z contains substituted or unsubstituted carbon or hetero atoms sufficient to form a ring. The preferred heteroatom is nitrogen. Most preferably, Z contains all carbon atoms. Preferred substituents on Z may be, for example, methyl, ethyl, or phenyl groups. R<sup>8</sup> is a substituted or unsubstituted alkyl or aryl group of 2 to 10 carbon atoms, and more preferably, 4 to 8 carbon atoms, or the free acid, alkaline earth salt, or the alkylammonium or arylammonium salt of the aforementioned groups. Preferably, R<sup>8</sup> is a substituted or unsubstituted carboxyalkyl, carboxyaryl, alkyl ester, or aryl ester group. Examples of appropriate substituents include alkyl and aryl groups.

More preferably, Z comprises four carbon atoms and R<sup>8</sup> is an alkyl or carboxyalkyl group of 4 to 8 carbon atoms, or the free acid, alkaline earth salt or ammonium salt of the aforementioned groups. The most preferred disulfide compounds of general Formula III are 5-thiocetic acid and 6-thiocetic acid. Examples of Formula III are the following:



(III-1)



(III-2)

-continued

(III-3)



The dichalcogenide compounds of this invention can be prepared by the various methods known to those skilled in the art.

10 Photographic emulsions are generally prepared by precipitating silver halide crystals in a colloidal matrix by methods conventional in the art. The colloid is typically a hydrophilic film forming agent such as gelatin, alginic acid, or derivatives thereof.

15 The crystals formed in the precipitation step are chemically and spectrally sensitized, as known in the art. Chemical sensitization of the emulsion employs sensitizers such as sulfur-containing compounds, e.g., allyl isothiocyanate, sodium thiosulfate and allyl thio-urea; reducing agents, e.g., polyamines and stannous salts; noble metal compounds, e.g., gold, platinum and diethylenide; and polymeric agents, e.g., polyalkylene oxides. A temperature rise is employed to complete chemical sensitization (heat spike). Spectral sensitization is effected with agents such as sensitizing dyes. For

20 color emulsions, dyes are added in the spectral sensitization step using any of a multitude of agents described in the art. It is known to add such dyes both before and after the heat spike.

25 After spectral sensitization, the emulsion is coated on a support. Various coating techniques include dip coating, air knife coating, curtain coating, and extrusion coating.

30 The dichalcogen compounds of this invention can be added to the vessel containing the aqueous gelatin salt solution before the start of the precipitation; they can also be added during precipitation to the salt solution, the silver nitrate solution, or from a separate jet directly into the kettle. Addition through the silver nitrate solution may be preferred in some cases because the dichalcogen compounds are more soluble in such a solution. However, there is some indication that greater activity may be achieved if the dichalcogens are added in the salt solution or directly to the vessel before the start of precipitation. The compounds can be added from the beginning or part-way-through precipitation, however, they must be added before the end of precipitation.

35 The dichalcogenide compounds of this invention can be added before or during the precipitation of the silver 40 halide emulsion using any technique suitable for this purpose. They can be added from solutions or as solids. For example, they can be dissolved in a suitable solvent and added directly to the precipitating solutions, or they can be added in the form of a liquid/liquid dispersion similar to the technique used with certain couplers. Examples of suitable solvents or diluents include methanol, ethanol, or acetone. Parameters such as temperature, stirring time, and other variables for precipitating conventional emulsions are known to those skilled in 45 the art.

50 It is believed that the most preferred method of addition may be as a solid particle dispersion added directly to the kettle. Unexpectedly, it had been found that addition of the dichalcogenides using this method results in 55 significantly greater antifogging activity. The aqueous, solid particle dispersions are prepared by milling an aqueous slurry of dichalcogenide and surfactant using known milling technology. Examples of suitable milling

equipment include a ball milling and a SWECO mill. Descriptions of other general milling techniques which may be used with this invention may be found in Patton, Temple C. *Paint Flow and Pigment Dispersion*, Second Edition, Wiley-Interscience, New York, 1979, hereafter referred to as Patton.

Examples of milling media are zirconium oxide beads or silicon carbide sand. The milling temperature may be room temperature or slightly higher (<30° C.). Appropriate surfactants include, among others, Triton® X-200 (Rohm & Haas Company, Philadelphia, Pa.) an alkylated arylpolyether sulfonate and other anionic surfactants.

Following milling, the slurry is separated from the media by coarse filtration. Generally, the slurry is then diluted to working strength with a gelatin solution, although it is not necessary to do so. As an alternative, the slurry can be used directly. Sonification may be used, if necessary, to break up aggregates. Alternatively, the slurry and beads can be diluted into a gelatin solution and the beads separated from the final dispersion by coarse filtration. Characterization of the final dispersion for dichalcogenide content may be made by spectrophotometric analysis and for particle size by microscopy. For additional description of this technique, see U.S. Pat. No. 5,217,859 Boettcher et al. incorporated herein by reference.

The optimal amount of the dichalcogenide compound to be added and the point of addition will depend on the desired final result, the type of emulsion, the degree of ripening, the structure of the dichalcogenide, and other variables. In general, the concentration of dichalcogenide which is adequate is from about  $1 \times 10^{-9}$  to about  $1 \times 10^{-2}$  mol/mol Ag, with  $1 \times 10^{-7}$  to  $1 \times 10^{-2}$  mol/mol Ag being preferred. The more preferred range which gives good antifogging without reducing sensitivity is  $1 \times 10^{-6}$  to  $3 \times 10^{-4}$  mol/mol Ag. The more preferred range for the growth modification properties is  $1 \times 10^{-5}$  to  $1 \times 10^{-3}$  mol/mo Ag.

Combinations of the dichalcogenide compounds may be added, i.e., two or more of Formula II or Formula III compounds, or a combination of Formula II and III compounds. The dichalcogenide compounds also may be added in combination with other antifoggants and finish modifiers.

The method of this invention is particularly useful with intentionally or unintentionally reduction sensitized emulsions. As described in *The Theory of the Photographic Process*, Fourth edition, T. H. James, Macmillan Publishing Company, Inc., 1977, pages 151-152, reduction sensitization has been known to improve the photographic sensitivity of silver halide emulsions. Reduction sensitization can be performed intentionally by adding reduction sensitizers, chemicals which reduce silver ions to form metallic silver atoms, or by providing a reducing environment such as high pH (excess hydroxide ion) and/or low pAg (excess silver ion).

During precipitation of a silver halide emulsion, unintentional reduction sensitization can occur when silver nitrate or alkali solutions are added rapidly or with poor mixing to form emulsion grains, for example. Also, silver halide emulsions precipitated in the presence of ripeners (grain growth modifiers) such as thioethers, selenoethers, thioureas, or ammonia tend to facilitate reduction sensitization.

The reduction sensitized silver halide emulsions, prepared as described in this invention, exhibit good photo-

graphic speed but usually suffer from undesirable fog and poor storage stability.

Examples of reduction sensitizers and environments which may be used during precipitation or spectrochemical sensitization to reduction sensitize an emulsion include ascorbic acid derivatives; tin compounds; polyamine compounds; and thiourea dioxide-based compounds described in U.S. Pat. Nos. 2,487,850; 2,512,925; and British Patent 789,823. Specific examples of reduction sensitizers or conditions, such as dimethylamineborane, stannous chloride, hydrazine, high pH (pH 8-11) and low pAg (pAg 1-7) ripening are discussed by S. Collier in *Photographic Science and Engineering*, 23,113 (1979).

Examples of processes for preparing intentionally reduction sensitized silver halide emulsions are described in EP 0 348934 A1 (Yamashita), EP 0 369491 (Yamashita), EP 0 371388 (Ohashi,), EP 0 396424 A1 (Takada), EP 0 404142 A1 (Yamada) and EP 0 435355 A1 (Makino).

The method of this invention is also particularly useful with emulsions doped with group VIII metals such as iridium, rhodium, iron and osmium, as described in *Research Disclosure*, December, 1989, Item 308119, published by Kenneth Mason Publications, Ltd., Dudley Annex, 12a North Street, Emsworth, Hampshire PO10 7DQ, ENGLAND. It is common practice in the art to dope emulsions with these compounds for improved photographic properties such as reciprocity, sensitivity, and contrast.

A general summary of the use of iridium in the sensitization of silver halide emulsions is contained in Carroll, "Iridium Sensitization: A Literature Review", *Photographic Science and Engineering*, Vol. 24, No. 6, 1980. The use of iridium in precipitating an emulsion for low intensity reciprocity control is described in U.S. Pat. No. 4,997,751 (Kim). The use of osmium in precipitating an emulsion is described in U.S. Pat. No. 4,933,272 (McDugle et al.).

In some cases, when such dopants are incorporated, emulsions show an increased fresh fog and a lower contrast sensitometric curve when processed in the color reversal E-6 process, as described in *The British Journal of Photography Annual*, 1982, pages 201-203.

The emulsions, doped as described above with Group VIII metals, when precipitated with dichalcogenide compounds show a dramatic decrease in fresh fog and higher contrast. The high temperature storage stability of the unexposed film is also improved by the practice of this invention by reducing the change in speed.

The emulsions which show the greatest growth modification response are the tabular, cubic, and octahedral emulsions. The dichalcogenide compounds of this invention tend to restrain the surface growth of the silver halide grains causing thinner and smaller grains.

Ripeners, for example, thioether, thiourea, thiocyanate, and ammonia may be used to control size and dispersity in cubic, cubo-octahedral, octahedral; tabular, and other morphologies. Such ripened emulsions can exhibit a lack of edge and corner definition due to the silver halide solvent effect which produces rounded grains. Another limitation inherent to ripened emulsions is an inability to produce sharp phase boundaries between areas of varying halide content. The dichalcogenide compounds of this invention are particularly useful with such ripened emulsions because they provide better phase separation and more uniform crystal growth.

Morphology is also a function of pAg. For AgBrI emulsions, octahedra emulsions having <111> faces are normally formed under conditions of excess bromide ion concentration (high pAg). As the excess bromide concentration is moved toward excess silver ion concentrations (lower pAg), the morphology proceeds from tabular→octahedral→cubo-octahedral→cubic. In other words, the morphology is dependent upon the pAg conditions during the emulsion precipitation for a given halide composition. The practice of this invention causes a shift in this relationship. For example, conditions that favor formation of cubic emulsions without dichalcogenide, produce cubo-octahedra emulsions with dichalcogenide; conditions which favor cubo-octahedra emulsion without dichalcogenide, produce octahedra with dichalcogenide. The use of the dichalcogenide provides a method of independent control of grain morphology at a given pAg.

The photographic elements of this invention can be non-chromogenic silver image forming elements. They can be single color elements or multicolor elements. Multicolor elements typically contain dye image-forming units sensitive to each of the three primary regions of the visible spectrum. Each unit can be comprised of a single emulsion layer or of multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer, e.g., as by the use of microvessels as described in Whitmore, U.S. Pat. No. 4,362,806 issued Dec. 7, 1982. The element can contain additional layers such as filter layers, interlayers, overcoat layers, subbing layers and the like.

In the following discussion of suitable materials for use in the emulsions and elements of this invention, reference will be made to *Research Disclosure*, December, 1989, Item 308119, published by Kenneth Mason Publications, Ltd., Dudley Annex, 12a North Street, Emsworth, Hampshire PO10 7DQ, ENGLAND, the disclosures of which are incorporated herein by reference. This publication will be identified hereafter by the term "Research Disclosure".

The silver halide emulsions employed in the elements of this invention can be either negative-working or positive-working. Examples of suitable emulsions and their preparation are described in *Research Disclosure* Sections I and II and the publications cited therein. Other examples of suitable emulsions are described in U.S. Pat. Nos. 4,997,751 (Kim) and 4,656,122 (Sowinski et al.) and U.S. application Ser. No. 699,869 (Kim et al.). Some of the suitable vehicles for the emulsion layers and other layers of elements of this invention are described in *Research Disclosure* Section IX and the publications cited therein.

The silver halide emulsions can be chemically and spectrally sensitized in a variety of ways, examples of

which are described in Sections III and IV of the *Research Disclosure*. The elements of the invention can include various couplers including, but not limited to, those described in *Research Disclosure* Section VII, paragraphs D, E, F and G and the publications cited therein. These couplers can be incorporated in the elements and emulsions as described in *Research Disclosure* Section VII, paragraph C and the publications cited therein.

The photographic elements of this invention or individual layers thereof can contain among other things brighteners (Examples in *Research Disclosure* Section V), antifoggants and stabilizers (Examples in *Research Disclosure* Section VI), antistain agents and image dye stabilizers (Examples in *Research Disclosure* Section VII, paragraphs I and J), light absorbing and scattering materials (Examples in *Research Disclosure* Section VIII), hardeners (Examples in *Research Disclosure* Section X), plasticizers and lubricants (Examples in *Research Disclosure* Section XII), antistatic agents (Examples in *Research Disclosure* Section XIII), matting agents (Examples in *Research Disclosure* Section XVI) and development modifiers (Examples in *Research Disclosure* Section XXI).

The photographic elements can be coated on a variety of supports including, but not limited to, those described in *Research Disclosure* Section XVII and the references described therein.

Photographic elements can be exposed to actinic radiation, typically in the visible region of the spectrum, to form a latent image as described in *Research Disclosure* Section XVIII and then processed to form a visible dye image, examples of which are described in *Research Disclosure* Section XIX. Processing to form a visible dye image includes the step of contacting the element with a color developing agent to reduce developable silver halide and oxidize the color developing agent. Oxidized color developing agent in turn reacts with the coupler to yield a dye.

With negative working silver halide, the processing step described above gives a negative image. To obtain a positive (or reversal) image, this step can be preceded by development with a non-chromogenic developing agent to develop exposed silver halide, but not form dye, and then uniformly fogging the element to render unexposed silver halide developable. Alternatively, a direct positive emulsion can be employed to obtain a positive image.

Development is followed by the conventional steps of bleaching, fixing, or bleach-fixing, to remove silver and silver halide, washing and drying.

The following examples are intended to illustrate, without limiting, this invention.

## EXAMPLES

The following compounds are utilized in the Examples.

Compound A = P-acetamido phenyl disulfide

Compound B = HO—CH<sub>2</sub>CH<sub>2</sub>—S—CH<sub>2</sub>CH<sub>2</sub>—S—CH<sub>2</sub>CH<sub>2</sub>—OH

Compound C = anhydro-5'-chloro-3,3'-bis(3-sulfopropyl)naptho{1,2-d}oxazolothiacyanine hydroxide triethylamine

Compound D = anhydro-5,3,3'-di-(3-sulfopropyl)naptho (1,2-d)thiazolothiacyanine hydroxide

Compound E = 3-Methyl benzothiazolium iodide

Compound F = sodium aurous (I) dithiosulfate

-continued

Compound G = sodium thiosulfate pentahydrate

Compound H = 4-hydroxy-6-methyl-1,3,3a,7-tetraazaindene

Compound I = Benzoic acid, 4-chloro-3-[(2-(4-ethoxy-2,5-dioxo-3-(phenyl)methyl-1-imidazolidinyl)-4,4'dimethyl-1,3-dioxopropyl)amino)dodecyl ester

Compound J = Benzothiazolium salt,  $\text{BF}_4(-)$ 

Hexanamide,2-[2,4-bis(1,1-dimethylpropyl)phenoxy]-N-[4-[(2,2,3,3,4,4,4-heptafluoro-1-oxobutyl)amino]-3-hydroxyphenyl]-



5-thioctic acid



6-thioctic acid

## Example 1

2.63% I bromoiodide tabular emulsions A (control) and B (invention) were precipitated by a double jet procedure. The following procedure produced 1 mole of total silver precipitation. 0.0082 mole of silver was nucleated for 1 minute with 2 N  $\text{AgNO}_3$  while maintaining the  $\text{pAg}$  at 9.2. This was done by adding a salt solution of 1.98 N  $\text{NaBr}$  and 0.02 N KI to a vessel filled with 818 cc of an aqueous solution containing 1.87 g/l bone gelatin, 2.5 g/l  $\text{NaBr}$ , 0.32 cc/l Pluronic 31R1 (tradename of BASF Wyandotte Corp.) and a block copolymer of ethylene oxide and propylene oxide, at a pH of 1.85 and a temperature of 55° C. After adjusting the  $\text{pAg}$  to 9.4 by  $\text{NaBr}$ , the temperature was raised to 75° C.; 13.85 cc of 0.77M  $(\text{NH}_4)_2\text{SO}_4$  was added, and the pH was brought to 10.5 by 2.5 N  $\text{NaOH}$ . After holding for 9 minutes, the  $\text{pAg}$  was adjusted to 8.6 by the addi-

tion of an aqueous gelatin solution containing 100 g/l bone gelatin and 0.11 cc/l Pluronic 31R1 and the pH was adjusted to 3.0. The emulsion was then grown at 55  $\text{pAg}$  8.4 for 64.6 minutes by accelerated flow rates of 1.6N  $\text{AgNO}_3$  and a salt solution of 1.66N  $\text{NaNO}_3$  and 0.0168N KI. At this point, which completed 71% of the total silver precipitation, a preformed  $\text{AgI}$  emulsion (0.05  $\mu\text{m}$ ) was added to make a total 2.63% of I. After 60 3 minutes, the remaining 29% of the total silver was precipitated with 1.6N  $\text{AgNO}_3$  and 3.5 N  $\text{NaBr}$  at  $\text{pAg}$  7.7 for 15.7 minutes. 0.1 mg/Ag mole of  $\text{K}_2\text{IrCl}_6$  was added after 75% of total silver precipitation. The resultant emulsion was washed by an ultrafiltration technique and the pH and  $\text{pAg}$  were adjusted to 5.5 and 8.2, respectively. For emulsion B, Compound A, dissolved in methanol, was added to the silver nitrate solution. Their grain size and thickness was compared as shown below:

| Emulsions     | *Compound A | Mean Size          | **COV | Mean Thickness      | ***AR | ****Tabularity |
|---------------|-------------|--------------------|-------|---------------------|-------|----------------|
| A (Control)   | None        | 2.70 $\mu\text{m}$ | 31%   | 0.135 $\mu\text{m}$ | 20.0  | 148            |
| B (Invention) | 24.4        | 1.74 $\mu\text{m}$ | 40%   | 0.125 $\mu\text{m}$ | 13.9  | 111            |

\*mg/mole silver

\*\*coefficient of variation of total grains population

\*\*\*Aspect Ratio = mean size/mean thickness

\*\*\*\*Aspect ratio/thickness

The unexpected decrease in grain size and thickness is attributed to the growth inhibition properties of Compound A. No significant change was observed when the concentration of Compound A was reduced to 2.44 mg/Ag mole.

Emulsion A was chemically sensitized with gold and sulphur, and spectrally sensitized to the blue region of

were grown for 55.8 minutes instead of 64.6 minutes at 10 pAg 9.2 before addition of AgI seed; (7) the final growth was at pAg 8.7 with 1.68N NaSr for 13.3 minutes instead of pAg 7.7 for 15.7 minutes; and (8) Iridium was not added. Compound A, dissolved in methanol, was added to emulsion D in AgNO<sub>3</sub> solutions. These emulsions were monodispersed.

| Emulsions     | *Compound A | Mean Size          | COV | Mean Thickness      | AR   | Tabularity |
|---------------|-------------|--------------------|-----|---------------------|------|------------|
| C (Control)   | None        | 1.13 $\mu\text{m}$ | 12% | 0.129 $\mu\text{m}$ | 8.8  | 69         |
| D (Invention) | 24.4        | 1.36 $\mu\text{m}$ | 14% | 0.105 $\mu\text{m}$ | 13.0 | 123        |

\*mg/mole silver

the spectrum. Emulsion B was sensitized with 5% more sensitizers than emulsion A.

60 mg/ft<sup>2</sup> of the sensitized emulsions were coated 25 with 1.75 g/silver mole of Compound H as a stabilizer, 160 mg/ft<sup>2</sup> of yellow coupler Compound I, and 220 mg/ft<sup>2</sup> of gelatin over an antihalation support.

The emulsion layer was protected by a gelatin over-coat and hardened. The coatings were exposed for 1 second with 3200K through a step wedge and Kodak Wratten filter Wr2B on a 1B sensitometer and processed to form positive images for six minutes in a color developer of the type described in the British Journal of Photography Annual, 1982, pages 201 to 203 (Kodak E6 reversal process). The speed (reversal) was determined at 0.3 below Dmax (maximum density). Fog was determined by developing a black and white image for four minutes followed by forming a negative color image as described for reversal process. After fresh testing, the coatings were kept in 120° F. and 50% relative humidity for 2 weeks for testing storage stability. Changes in Dmax and speed due to the keeping condition are expressed as % Dmax and Dspeed.

Thickness reduction was noticeable and thereby tabularity was increased by the use of Compound A.

Emulsions C and D were sensitized with 100 mg NaCNS, 1013 mg Compound C, 4.4 mg Compound F, 2.18 mg Compound G and 24.2 mg Compound J for one mole of silver at 68° C. for 20 minutes. The emulsions were coated and evaluated as in Example 1 except that they were exposed at 1/50 seconds 5500K. The results shown below indicate that speed change upon keeping was reduced by the use of Compound A.

| Emulsions     | *Compound A | *Com- |      |       |        |        |
|---------------|-------------|-------|------|-------|--------|--------|
|               |             | Fog   | Dmax | Speed | % Dmax | Dspeed |
| C (Control)   | None        | 0.04  | 2.43 | 182   | -2     | +19    |
| D (Invention) | 24.36       | 0.04  | 2.41 | 182   | -2     | +8     |

\*mg/mole silver

### Example 3

A 5% I AgBrI cubic emulsion (Emulsion E) was made via a double jet method. 9 moles of silver halide emulsion were made at constant pAg 7.97 by varying the flow of the salt solution. The silver and salt solutions were added over a period of 35 minutes in a stirred kettle containing 8.3 liters of an aqueous 2% gelatin solution with 900 mg of ripener Compound B. The emulsion was desalinated by an ultrafiltration washing technique. The resultant emulsion grains showed perfect cubic structure and were measured to be 0.111  $\mu\text{m}$  (equivalent spherical diameter).

Emulsion F (Invention) was prepared like Emulsion E except a silver nitrate solution containing 24 mg/Ag mole of Compound A dissolved in methanol was added. Unexpectedly, the grains became rounded in the presence of Compound A. The size of the grain was 0.115  $\mu\text{m}$  and the grains lost their cubic characteristics by about 16% when estimated by dye adsorption method similar to the procedure described by H. Philippaerts, et al., Journal of Photographic Science, Vol. 20, p. 215 (1972) and T. Tani, "Journal of Imaging Science, Vol. 29, p. 165 (1985). Therefore, Compound A appeared to restrain <111> surface growth.

| Emulsions     | *Compound A | *Com- |      |       |        |        |
|---------------|-------------|-------|------|-------|--------|--------|
|               |             | Fog   | Dmax | Speed | % Dmax | Dspeed |
| A (Control)   | None        | 0.11  | 1.51 | 205   | -15    | +18    |
| B (Invention) | 24.4        | 0.05  | 1.95 | 188   | -4     | +6     |

\*mg/mole silver

Less speed change and Dmax loss on keeping and fresh fog reduction were obtained by the addition of Compound A in the precipitation. In addition, there was no change in latent image stability.

### Example 2

2.68% I bromoiodide monodispersed tabular emulsions C (control) and D (invention) were similarly precipitated as described in Example 1 with the following modifications: (1) the level of Fluoronic 31R1 in the initial vessel was reduced to 0.11 cc/l; (2) the temperatures for nucleation and growth were 45° C. and 60° C., respectively; (3) the pAg of nucleation was 9.7 and was adjusted to 9.8 before addition of gelatin solution to pAg 9.2; (4) the pH for the ammonia digest was 9.5; (5) the pH for growth was 5.8; (6) the nucleated emulsions

The emulsions were chemically sensitized with sulphur and gold, spectrally sensitized to the red region spectrum, and coated with gelatin and cyan dye forming coupler and then evaluated as described in Example 1, except the images were developed for four minutes. Photographic results are shown below. Contrast is an average gamma. Ddmax is change in Dmax.

| Emulsions     | A    | *Compound |       |      |       |
|---------------|------|-----------|-------|------|-------|
|               |      | Fog       | Speed | Dmax | DDmax |
| E (Control)   | None | 0.72      | 276   | 1.00 | -.46  |
| F (Invention) | 24.0 | 0.11      | 245   | 1.57 | -.11  |

\*mg/mole silver

The fog reduction by Compound A made the emulsion acceptable in terms of photographic utility: higher contrast and good keeping (less Dmax loss and speed gain).

#### Example 4

For reciprocity control, the emulsions described in Example 3 were doped with varying levels of K<sub>2</sub>IrCl<sub>6</sub> as disclosed in U.S. Pat. No. 4,902,611 (Leubner and White, 1990) as shown below:

| Emulsion | Ir*  | Compound A* | Size  | Fog  | Speed | Contrast | Ddmax | Dspeed |
|----------|------|-------------|-------|------|-------|----------|-------|--------|
| G        | 0.30 | 0.8         | 0.117 | 1.03 | 281   | 0.59     | -.20  | +.13   |
| H        | 0.05 | 0.8         | 0.113 | 0.80 | 287   | 0.91     | -.22  | +.11   |
| I        | 0.15 | 12.0        | 0.113 | 0.57 | 260   | 1.51     | -.15  | +.16   |
| J        | 0.30 | 24.0        | 0.108 | 0.08 | 238   | 1.42     | -.14  | +.18   |
| K        | 0.05 | 24.0        | 0.107 | 0.22 | 243   | 1.54     | -.15  | +.11   |
| L        | 0.15 | 24.0        | 0.112 | 0.28 | 243   | 1.51     | -.14  | +.13   |
| M        | 0.15 | 24.0        | 0.113 | 0.25 | 247   | 1.46     | -.14  | +.11   |

\*in mg/silver mole

Increase in fresh fog and lower contrast due to iridium were improved by the introduction of Compound A. As the level of Compound A increased, the change in Dmax due to keeping was also improved and relative 40 cubic characters was decreased.

#### Example 5

Emulsion N (Invention) was made as follows. The starting kettle contained 6 liters of water, 90 g of gel, 45 30.4 g of (NH<sub>4</sub>)<sub>2</sub>SO<sub>4</sub>, and 6.4 g of NaBr, at 80° C. The pH of the kettle was adjusted to 10.0 before the start of the precipitation. 24 mg of Compound A, dissolved in methanol, per silver mole was added to all AgNO<sub>3</sub> solutions. A double-jet run of 0.021 mole of AgNO<sub>3</sub> and NaBr was added over a time period of 1.2 minutes controlling the pAg at 8.0. The kettle was held for 1 minute. Then 5.25 moles of AgNO<sub>3</sub> and 4.2 moles of NaBr and 1.05 mole of KI were added via a double-jet method into the kettle over a time period of 65.6 minutes. The kettle was held for 10 minutes and the pH adjusted from 10 to 5.5 during that time. The run continued with addition of 0.45 mole of AgNO<sub>3</sub> and NaBr in an unbalanced flow with faster AgNO<sub>3</sub> addition to change the pAg from 8.0 to 6.3 in a time period of 6 minutes. The run continued with 4.8 moles of AgNO<sub>3</sub> and NaBr over 48.5 minutes controlling pAg at 6.3. The emulsion was de-salted, pAg was adjusted to 7.6 and pH was adjusted to 5.75. The emulsion had an ECD (equivalent circular diameter) of 1.6 μm and consisted of all octahedral 55 grains.

A comparative example, Emulsion O was made without the addition of Compound A to the AgNO<sub>3</sub> solu-

tions. The emulsion was 1.7 μm and contained all cubooctahedra grains.

The x-ray powder diffraction study (XRPD) showed that the invention has a lower iodide containing shell and that the invention has more uniform iodide in both the core and shell as indicated by the narrower full width half maximum (FWHM) as shown below:

| Emulsions     | ECD    | Shape    | % I:FWHM Core | % I:FWHM Shell |
|---------------|--------|----------|---------------|----------------|
| N (Invention) | 1.7 μm | octa     | 19.7:0.18     | 0.4:0.26       |
| O (Control)   | 1.6 μm | cuboocta | 19.4:0.20     | 1.6:0.36       |

15 The emulsions were chemically sensitized with sulphur and gold. The sensitized emulsions were coated with gelatin and yellow dye forming coupler on a support. The emulsion was stabilized with Compound H. The emulsion layer was protected by a gelatin overcoat and hardened. The coatings were exposed through a step wedge on a 1B sensitometer and processed in Kodak color negative C-41 process.

| Emulsions     | Fog  | *Speed | Dmax |
|---------------|------|--------|------|
| N (Invention) | 0.11 | 100    | 1.8  |

| O (Control)      | 0.97 | 100 | 1.8 |
|------------------|------|-----|-----|
| *0.15 above Dmin |      |     |     |

The invention having Compound A reduced the fog considerably without altering speed and Dmax.

#### Example 6

0.2 micrometer cubic AgCl emulsions P through S were precipitated with Compound A (0.8 mg/mole Ag) added in a variety of ways.

#### Emulsion P

An AgCl cubic emulsion was made via a double jet method. 9 moles of silver halide were made at a constant pAg of 7.55 by varying the flow of the salt solution. The silver and salt were added over a period of 25 minutes in a stirred kettle containing 7.2 liters of an aqueous 2.5% gelatin solution. The emulsion was de-salted by an ultrafiltration technique.

#### Emulsion O

Emulsion Q was prepared in a similar manner except that 0.8 mg/Ag mole of Compound A was dissolved in methanol and was added to the 3N AgNO<sub>3</sub> solution used to prepare the emulsion.

#### Emulsion R

Emulsion R is the same as Emulsion Q except that the methanolic solution of Compound A was added to the 3N NaCl solution used to prepare the emulsion instead of the 3N AgNO<sub>3</sub> solution.

## Emulsion S

Emulsion S was the same as Emulsion P except the methanolic solution of Compound A was added to the precipitation kettle before the start of the emulsion precipitation.

The resulting emulsions were sulfur plus gold sensitized, dyed with a sensitizing dye (Compound K) and tested in a black-and-white developer KODAK DK-50. Toe speed was measured at 0.1 above Dmin.

| Emulsions     | Where Added          | Toe Speed | Fog  |
|---------------|----------------------|-----------|------|
| P (Control)   | none                 | 2.54      | 0.44 |
| Q (Invention) | 3N AgNO <sub>3</sub> | 2.56      | 0.35 |
| R (Invention) | 3N NaCl              | 2.31      | 0.06 |
| S (Invention) | Kettle               | 2.34      | 0.06 |

Compared to the control emulsion, the addition of Compound A during precipitation reduced fog.

## Example 7

Pure silver chloride cubic emulsions T through Y were precipitated by equimolar addition of 3.8 molar silver nitrate and sodium chloride solutions into a reactor containing 195 g of bone gelatin, 35.9 g of sodium chloride, 6969 ml of distilled water, and Compound B at a temperature of 68.3° C. Initial temperature and pAg was maintained constant throughout the precipitation. Feed solution flows and the amount of ripener (Compound B) were adjusted to obtain 0.72 micrometer silver chloride cubes. Various levels of Compound A, dissolved in methanol, were added to the AgNO<sub>3</sub> feed solution. The extent of reduction sensitized fog was

To a precipitation vessel was added 6.72 l of a distilled water solution that was 546.4 g sodium bromide, 26.72 g potassium iodide, and contained 248 g bone gelatin. The solution was stirred and pH was measured at 5.77 at 40° C. The temperature was increased to 79° C. A 1.5 molar silver nitrate solution was added through a jet at a constant flow for 41 minutes with 8 moles of silver added. A 3 molar sodium bromide solution was added through a second jet with the following flow rates for a total of 41 minutes; 0.071 moles for 2.5 minutes, 0.51 moles for 10 minutes with increasing flow rate of 1.52x, 0.40 moles for 5 minutes with increasing flow rate of 0.68x, 0.43 moles for 5 minutes with increasing flow rate of 0.22x, 0.46 moles for 5 minutes with increasing flow rate of 0.7x, and 0.69 moles for 8.5 minutes with decreasing flow rate of -1.271x. At the end of the silver run, 100 cc of aqueous ammonium sulfate solution (0.17 g/ml) was added into the vessel followed by addition of 6.5 ml/Ag mole of 15N ammonium hydroxide solution. After holding for 5 minutes, pH was adjusted to 6.0 and the emulsion was washed.

Due to the ammonia digestion, these emulsions are prone to reduction sensitization fog. To lower fog, Compound A, dissolved in methanol, was added through the silver nitrate solutions. Grain size of the emulsions was 1.63 μm and 1.5 μm for Emulsions Z and CC, respectively. Both emulsions were sensitized with sulfur, gold and blue spectral sensitizer Compound C. For comparison, Compound A was added to the sensitized emulsion Z prior to coating as described in U.S. Pat. No. 3,397,986. Coatings were prepared and evaluated as described in Example 1, except that 89 mg/ft<sup>2</sup> silver and 180 mg/ft<sup>2</sup> Compound I were coated. The results are shown below:

| Emulsions      | *Compound A | Where Added   | Fog  | Dmax | Speed | Contrast |
|----------------|-------------|---------------|------|------|-------|----------|
| Z (Control)    | none        | none          | 1.63 | 0.15 | 0     | 0        |
| AA (Control)   | 24          | melt          | 1.61 | 0.21 | 0     | 0        |
| BB (Control)   | 90          | melt          | 1.59 | 0.23 | 0     | 0        |
| CC (Invention) | 24          | precipitation | 0.42 | 1.43 | 215   | -149     |

\*in mg/silver mole

determined by adding 4 mg KAuCl<sub>4</sub> per mole of silver followed by a heat digestion at 60° C. for 55 minutes. The reduction sensitized fog was reduced by the addition of Compound A as shown below:

| Emulsion Number | Compound A* | Fog  |
|-----------------|-------------|------|
| T (Control)     | 0.0         | 0.18 |
| U (Invention)   | 0.4         | 0.15 |
| V (Invention)   | 4           | 0.13 |
| W (Invention)   | 8           | 0.10 |
| X (Invention)   | 20          | 0.08 |
| Y (Invention)   | 40          | 0.06 |

\*mg/silver mole

As the concentration of Compound A increased, reduction sensitized fog was reduced.

## Example 8

Iridium doped 2% I bromoiodide emulsions digested with ammonia were prepared by the following procedure.

The control emulsion Z showed too high fog to determine speed and contrast. The comparative coatings, AA and BB prepared as taught by Millikan and Herz (U.S. Pat. No. 3,397,986) did not reduce fog significantly. Only when added to the emulsion during precipitation, did Compound A provide acceptable photographic results (fog, Dmax, and speed).

Kodak C-41 Color negative process of the above coatings provided similar conclusions as for the Kodak E6 process:

| Emulsions      | Fog  | *Speed |
|----------------|------|--------|
| Z (Control)    | 0.98 | 246    |
| AA (Control)   | 1.00 | 231    |
| BB (Control)   | 0.98 | 220    |
| CC (Invention) | 0.18 | 264    |

\*contrast normalized speed

65 The mode of spectral sensitization was not important. Emulsions Z and CC were sensitized by adding blue spectral sensitizer Compound C before and after heat digestion.

| Emulsions      | Sensitization    | % fog** | Dmax | Speed | % Dmax | Dspeed | # LIK |
|----------------|------------------|---------|------|-------|--------|--------|-------|
| Z (Control)    | 67 C. 20 min/dye | 92      | 0.25 | 0     | *      | *      | *     |
| AA (Invention) | 67 C. 20 min/dye | 19      | 2.27 | 237   | -8%    | 2      | -5    |
| BB (Control)   | dye/73 C. 20 min | 76      | 0.7  | 219   | *      | *      | *     |
| CC (Invention) | dye/73 C. 20 min | 19      | 2.26 | 234   | -17%   | -9     | +4    |

\*not measurable due to high fog

\*\*percent silver fogged of total silver coated

# Latent image keeping speed change at 78 F. and 50% relative humidity for 2 weeks

Regardless of how Emulsion CC was spectrally sensitized, when doped with Compound A during precipitation it provided lower fresh fog and fog growth during high temperature keeping, and acceptable LIK.

#### Example 9

Fine 3.4% I bromoiodide Emulsions, DD and EE were prepared similarly as described in Example 8 with a lower temperature of 44° C., higher iodide of 3.4% I, and 28 minute precipitation time. Similar fog reduction was observed as in Example 8.

| Emulsions      | *Compound A | Size, $\mu\text{m}$ | Fog  | Speed |
|----------------|-------------|---------------------|------|-------|
| DD (Control)   | none        | 0.364               | 0.21 | 325   |
| EE (Invention) | 24          | 0.342               | 0.14 | 323   |

\*mg/silver mole

#### Example 10

Fine grain 4.8% I bromoiodide core/shell emulsions FF through JJ were precipitated in a reactor containing ammonia before the start of the precipitation. After growing crystals in the presence of the ammonia for a desired period, pH was adjusted to below 6. Then  $\text{AgNO}_3$  and  $\text{NaBr}$  salt were added in order to grow crystals further at a desired pAg. A methanolic solution of Compound A was added to the  $\text{AgNO}_3$  solution throughout precipitation. Due to the high pH of the added ammonia, these emulsions are prone to reduction sensitization fog. The emulsions were sensitized with blue or red sensitizing dyes and tested as described in Example 1. The fog reduction by Compound A was apparent.

| Emulsions      | Sens | Size, $\mu\text{m}$ | *Compound A | Speed | Fog  |
|----------------|------|---------------------|-------------|-------|------|
| FF (Control)   | Blue | 0.154               | 0           | 192   | 0.57 |
| GG (Invention) | Blue | 0.155               | 24          | 181   | 0.19 |
| HH (Control)   | Red  | 0.159               | 0           | 242   | 0.22 |
| II (Invention) | Red  | 0.156               | 0.8         | 247   | 0.13 |
| JJ (Invention) | Red  | 0.156               | 24          | 245   | 0.09 |

\*mg/silver mole

#### Example 11

0.44  $\mu\text{m}$  2% I bromoiodide emulsions KK, LL, and MM were prepared similarly as described in Example 9, except that iridium was added after 90% of the total silver precipitation and ammonia digestion was not performed. The emulsions were sensitized with 42 mg  $\text{NaSCN}$ , 22 mg Compound E, 7.0 mg sodium thiosulfate pentahydrate, and 3.5 mg potassium tetrachloroaurate (all per mole Ag) at 70° C. for 20 minutes. Red sensitizing dye (Compound L) was added, coated with cyan dye forming coupler (Compound M), and tested as described in Example 1.

| Emulsions      | *Compound A | Fog  | Dmax | Speed | % Dmax | Dspeed |
|----------------|-------------|------|------|-------|--------|--------|
| KK (Control)   | None        | 0.35 | 2.00 | 246   | -81    | -68    |
| LL (Invention) | 12          | 0.25 | 2.15 | 245   | -51    | -26    |
| MM (Invention) | 24          | 0.26 | 2.15 | 250   | -47    | -29    |

\*mg/silver mole

Compound A, when added in the precipitation, provided significant reductions in fresh fog without speed loss, and significantly less fog growth (less %Dmax loss) as well as less speed loss when coatings were stored at 120° and 50% relative humidity for 2 weeks.

#### Example 12

Emulsions NN through PP were prepared as described in Example 7, except that after the initial 5 minutes of the double-jet precipitation, a silver solution containing various amounts of 5-thioc acid (Compound N) and 6-thioc acid (Compound O) dissolved in methanol was used. The emulsions were sensitized with 280 mg of blue sensitizing dye (Compound D), 0.75 g  $\text{KBr}$ , 2.5 mg sodium thiosulfate pentahydrate, and 1.25 mg potassium tetrachloroaurate (per silver mole) at 80° C. for 20 minutes. After heat ramp, 86 mg of 1-(3-acemidophenyl)-5-mercaptopetrazole per silver mole was added. The emulsions were coated on a paper support and were processed in Kodak RA-4 chemistry (Research Disclosure Vol 308, 1989, p 933. Speed was taken at density=1.

| Emulsions      | Addendum*          | Fog  | Speed | Contrast |
|----------------|--------------------|------|-------|----------|
| NN (Control)   | none               | 0.16 | 122   | 1.22     |
| OO (Invention) | Compound N at 0.01 | 0.09 | 117   | 1.66     |
| PP (Invention) | Compound O at 0.01 | 0.07 | 113   | 1.83     |

\*concentrations in mmole per silver mole

At the most preferred concentration, 0.01 mmole per silver mole, unacceptable high fog was reduced by both compounds N and O to practical levels for color paper applications.

#### Example 13

Emulsions QQ through WW were prepared as described in Example 12, except that higher concentrations of 5-thioc acid (Compound N) were used.

| Emulsion | Compound N* | Size  | Shape                      | Figure |
|----------|-------------|-------|----------------------------|--------|
| QQ       | 0           | 0.728 | rounded cube               |        |
| RR       | 0.010       | 0.743 | rounded cube               |        |
| SS       | 0.060       | 0.737 | cubooctahedra              |        |
| TT       | 0.120       | 0.715 | cubooctahedra              |        |
| UU       | 0.322       | 0.693 | cubooctahedra              |        |
| VV       | 0.970       | 0.729 | cubooctahedra + (110) edge |        |
| WW       | 2.910       | 0.727 | cubooctahedra +            |        |

-continued

| Emulsion | Compound N* | Size | Shape      | Figure |
|----------|-------------|------|------------|--------|
|          |             |      | (110) face |        |

\*concentrations are in mmole per silver mole

5-thioctic acid affects the growth of (111) and (110) crystallographic faces at the same time, leading to the morphology with all those faces present (at concentration of 2.91 mmol/Ag mol). At lower concentrations (0.3-1 mmol/Ag mol), well-developed cubooctahedra are formed, whereas at yet lower concentrations the share of (111) face is decreasing down to that of the control emulsion QQ prepared without the Compound N.

## Example 14

AgCl Emulsions XX through AAA were prepared as described in the Example 7 except that  $2 \times 10^{-6}$  g of dicesium pentachloro nitrosoyl osmate per silver mole was added through the salt solutions as described by McDugle, et al., U.S. Pat. No. 4,933,272. The amount of Compound A added to each silver nitrate solution and the resulting fog levels (tested as described in Example 7) are shown below.

| Emulsions       | *Compound A | Fog  |
|-----------------|-------------|------|
| XX (Control)    | None        | 0.29 |
| YY (Invention)  | 0.2         | 0.20 |
| ZZ (Invention)  | 0.4         | 0.16 |
| AAA (Invention) | 0.8         | 0.16 |

\*mg/Ag mole

As shown above, Compound A reduced fog in AgCl emulsions doped with osmium.

While the invention has been described in detail and with reference to specific embodiments thereof, it will be apparent to one skilled in the art that various changes and modifications can be made therein without departing from the spirit and scope thereof.

## Example 15

A pure silver chloride emulsion (Emulsion BBB, Control) was precipitated by a double jet technique with the use of 1,8-dithiaoctanediol as ripener. The 45 resultant cubic emulsion had 0.75  $\mu\text{m}$  edgelength. It was then chemically and spectrally sensitized, as described below. In another emulsion (Emulsion CCC, Control) prepared, as described above, mercuric chloride was added to the silver feed solution. This emulsion was sensitized, as described below.

Two other emulsions, (Emulsion DDD & EEE), were prepared, as described above, but after the initial 5 minutes of precipitation, a silver solution containing various amounts of 6-thioctic acid (Compound O), dissolved in methanol, were added. With this addition, the usual rounded cubic morphology with a higher percentage of (111) crystallographic face at the corners changed to a much sharper cubic morphology bounded almost exclusively by (100) crystallographic faces.

All of the emulsions were sensitized by the addition of gold sulfide and ripening for 65 minutes at an elevated temperature, during which time a cyanine yellow sensitizing dye was introduced as well as 1-(3-acetomidophenyl)-5-mercaptopetrazole and potassium bromide. Sodium chloride was added to all the emulsions prior to coating. Immediately prior to coating, the emulsions were dual mixed with a yellow coupler dis-

persion which was stabilized by benzenosulfonic acid. All of the emulsions were coated at 26 mg of silver, 100 mg of yellow coupler and 77 mg of gelatin per square foot on a resin coated paper support and were subsequently subjected to sensitometric gradation exposure through a set of Kodak filters. The exposure time was 1/10 second. Processing was by the rapid access Kodak RA-4 process, as described in Research Disclosure, Vol. 308, p. 933, 1989. Speed was measured by 1.0 density.

TABLE 1

| Emulsion           | Compound O<br>( $\mu\text{mole/Ag Mole}$ ) | Photographic Properties |       |                                       |              |
|--------------------|--------------------------------------------|-------------------------|-------|---------------------------------------|--------------|
|                    |                                            | Fresh                   |       | Incubation<br>3 Day/<br>100° F./50 RH |              |
|                    |                                            | Speed                   | Fog   | $\Delta$ Speed                        | $\Delta$ Fog |
| BBB<br>(Control)   | 0                                          | 209                     | 0.160 | 9                                     | 0.060        |
| CCC<br>(Control)   | 0                                          | 209                     | 0.070 | 9                                     | 0.105        |
| DDD<br>(Invention) | 1.0                                        | 206                     | 0.065 | 12                                    | 0.065        |
| EEE<br>(Invention) | 0.1                                        | 206                     | 0.140 | 10                                    | 0.080        |

## Example 16

Emulsion FFF (Invention) and Emulsion GGG (Invention) were made as follows. The starting kettle contained 6 liters of water, 90 g of gel, 30.4 g of  $(\text{NH}_4)_2\text{SO}_4$ , and 6.4 g of NaBr, at 80° C. The pH of the kettle was adjusted to 10.0 before the start of the precipitation. A double-jet run of 0.021 mole of  $\text{AgNO}_3$  and NaBr was added over a time period of 1.2 minutes controlling the pAg at 8.0. The kettle was held for 1 minute. Then 5.25 moles of  $\text{AgNO}_3$  and 4.2 moles of NaBr and 1.05 mole of KI were added via a double-jet method into the kettle over a time period of 65.6 minutes. The kettle was held for 10 minutes and the pH adjusted from 10 to 5.5 during that time. The run continued with addition of 0.45 mole of  $\text{AgNO}_3$  and NaBr in an unbalanced flow with faster  $\text{AgNO}_3$  addition to change the pAg from 8.0 to 6.3 in a time period of 6 minutes. The run continued with 4.8 moles of  $\text{AgNO}_3$  and NaBr over 48.5 minutes controlling pAg at 6.3. The emulsion was desalted, pAg was adjusted to 7.6 and pH was adjusted to 5.75. The emulsion had an ECD (equivalent circular diameter) of 1.6  $\mu\text{m}$  and consisted of all cubo-octahedral grains. For Emulsion FFF, 1 mg of Compound A/mol Ag was added to all of the salt solutions except the silver salt solutions. For Emulsion GGG, 40 mg of Compound A was dissolved in 10 cc of methanol and added as a dump after the NaBr and KI addition and before the pH adjustment.

A comparative example, Emulsion HHH (Control) was made without the addition of Compound A. The emulsion was 1.7  $\mu\text{m}$  and contained all cubo-octahedral grains.

The x-ray powder diffraction study (XRPD) showed that the invention (Emulsion GGG), which had the addition of Compound A after the BrI core, has a lower iodide containing shell and that the invention (Emulsion FFF), with the addition of Compound A during the whole time of the make, has more uniform iodide in both the core and shell as indicated by the narrower full width half maximum (FWHM) as shown below. These two examples clearly show that Compound A is the

factor causing the change in FWHM and the more uniform iodine distribution.

where G is independently in an ortho, meta, or para position on the aromatic nucleus relative to the sulfur and is hydrogen, hydroxy,  $\text{SO}_3\text{M}$  or  $\text{NR}^3\text{R}^4$ ; M is hydrogen, or an alkaline earth, alkylammonium or arylammonium cation; R<sup>3</sup> is hydrogen, or a substituted or unsubstituted alkyl or aryl group;

| Emulsion        | ECD               | Shape     | % I:FWHM   | % I:FWHM  | Fog  | Speed | Dmax |
|-----------------|-------------------|-----------|------------|-----------|------|-------|------|
| FFF (Invention) | 1.6 $\mu\text{m}$ | cubo-octa | 19.9:0.179 | 1.3:0.294 | 0.21 | 95    | 1.8  |
| GGG (Invention) | 1.6 $\mu\text{m}$ | cubo-octa | 19.5:0.206 | 1.1:0.295 | 0.44 | 98    | 1.8  |
| HHH (Control)   | 1.6 $\mu\text{m}$ | cubo-octa | 19.4:0.200 | 1.6:0.360 | 0.97 | 100   | 1.8  |

The emulsions were chemically sensitized with sulphur and gold. The sensitized emulsions were coated with gelatin and yellow dye forming coupler on a support. The emulsion was stabilized with Compound H. The emulsion layer was protected by a gelatin overcoat and hardened. The coatings were exposed through a 25 step wedge on a 1B sensitometer and processed in Kodak color negative C-41 process.

The invention having Compound A reduced the fog considerably without altering speed and Dmax.

What is claimed is:

1. A method of making a photographic silver halide emulsion comprising:  
precipitating a silver halide emulsion; and  
adding to the silver halide emulsion before or during  
precipitation a non-labile chalcogen compound 35  
represented by Formula I:



(Formula I)

where  $\text{X}^1$  and  $\text{X}^2$  are independently S, Se, or Te; and 40  
 $\text{R}^1$  and  $\text{R}^2$ , together with  $\text{X}^1$  and  $\text{X}^2$ , form a ring system, or are independently substituted or unsubstituted cyclic, acyclic or heterocyclic groups.

2. The method of claim 1 wherein  $\text{R}^1$  and  $\text{R}^2$  are independently substituted alkyl or aryl groups; the dichalcogenide molecule is symmetrical and the molecular weight is greater than 210 g/mol.

3. The method of claim 1 wherein the dichalcogenide compound is a disulfide compound represented by Formula II or III:



(Formula II)

5

$\text{R}^4$  is hydrogen,  $\text{O}=\text{C}-\text{R}^5$ , or  $\text{O}=\text{C}-\text{N}-\text{R}^6\text{R}^7$ ; and  $\text{R}^5$ ,  $\text{R}^6$ , and  $\text{R}^7$  are independently hydrogen, or hydroxy, or an unsubstituted alkyl, or aryl group, or a substituted or unsubstituted fluoroalkyl, fluoroaryl, carboxyalkyl, carboxyaryl, alkylthioether, arylthioether, sulfoalkyl, or sulfoaryl group or the free acid, alkaline earth salt or alkylammonium or arylammonium salt of the aforementioned groups,

30

(Formula III)



where Z contains substituted or unsubstituted carbon or hetero atoms sufficient to form a ring; and  $\text{R}^8$  is a substituted or unsubstituted alkyl or aryl group of 2 to 10 carbon atoms, or the free acid, alkaline earth salt, arylammonium or alkylammonium salt of the aforementioned groups.

45 4. The method of claim 3 wherein the disulfide is represented by Formula II and the molecule is symmetrical and G is in an ortho, meta, or para position on the aromatic nucleus relative to the sulfur and is  $\text{NR}^3\text{R}^4$ , and  $\text{R}^4$  is hydrogen, or  $\text{O}=\text{C}-\text{R}^5$ .

50 5. The method of claim 4 wherein G is in a para position relative to sulfur,  $\text{R}^3$  is hydrogen or methyl,  $\text{R}^4$  is  $\text{O}=\text{C}-\text{R}^5$  and  $\text{R}^5$  is an alkyl group of 1 to 10 carbon atoms, an aryl group of 6 to 10 carbon atoms or a trifluoromethyl group.

55 6. The method of claim 5 wherein the disulfide compound is p-acetamidophenyl disulfide.

60 7. The method of claim 3 wherein the disulfide compound is represented by Formula III and  $\text{R}^8$  is a substituted or unsubstituted carboxyalkyl, carboxyaryl, alkyl ester, or aryl ester group of 2 to 10 carbon atoms, or the free acid, alkaline earth salt, arylammonium or alkylammonium salt of the aforementioned groups.

65 8. The method of claim 7 wherein Z comprises carbon atoms sufficient to form a ring and  $\text{R}^8$  is a substituted or unsubstituted alkyl or aryl group of 4 to 8 carbon atoms, or the free acid, alkaline earth salt, ary-

lammonium or alkylammonium salt of the aforementioned groups.

9. The method of claim 8 wherein R<sup>8</sup> is a substituted or unsubstituted carboxyalkyl, carboxyaryl, alkyl ester, or aryl ester group of 4 to 8 carbon atoms, or the free acid, alkaline earth salt, arylammonium or alkylammonium salt of the aforementioned groups.

10. The method of claim 9 wherein the disulfide compound is 5-thioctic acid or 6-thioctic acid.

11. The method of claim 3 wherein the amount of the disulfide compound added is  $1 \times 10^{-7}$  to  $1 \times 10^{-2}$  mol/mol Ag.

12. The method of claim 3 wherein the amount of the disulfide compound added is  $1 \times 10^{-6}$  to  $3 \times 10^{-4}$  mol/mol Ag.

13. The method of claim 3 wherein the amount of the disulfide compound added is  $10^{-5}$  to  $10^{-3}$  mol/mol Ag.

14. The method of claim 3 wherein the silver halide emulsion is a reduction sensitized emulsion.

15. The method of claim 3 wherein the silver halide emulsion is doped with a Group VIII metal.

16. The method of claim 3 wherein the silver halide emulsion is precipitated in the presence of ripeners.

17. The method of claim 1 wherein precipitating the silver halide emulsion comprises adding at least one non-silver salt solution to the emulsion and wherein the dichalcogenide compound is first added to the non-silver salt solution and the dichalcogenide containing salt solution is then added to the emulsion.

18. A photographic silver halide emulsion prepared by the method described in any one of claims 1 through 17.

\* \* \* \* \*

20

25

30

35

40

45

50

55

60

65